

## UNITED STATES PATENT OFFICE

2,615,837

## ELECTROPLATING BATH AND PROCESS

Andrew W. Liger, Wyandotte, Mich., assignor to  
Wyandotte Chemicals Corporation, Wyandotte,  
Mich., a corporation of Michigan

No Drawing. Application November 20, 1947,  
Serial No. 787,255

5 Claims. (Cl. 204—49)

The present invention relates to an electroplating composition and process. The general object and nature of my invention is to provide an electroplating solution which will impart a bright finish to the metal deposited. My invention is based on the discovery that sodium carboxymethylcellulose (also called "sodium cellulose glycolate") acts as a brightening agent in metal plating baths, particularly in the electroplating of nickel and cadmium.

Only a relatively small proportion of the sodium carboxymethylcellulose brightening agent is required to be added to the plating bath. The amount of sodium carboxymethylcellulose additive has been found to be in the range of 0.05—2.50% by weight of the electroplating solution.

The following examples serve to illustrate my invention in detail and better to aid those skilled in the art in the understanding of same.

## EXAMPLE 1

A nickel plating bath was made up of the following composition:

|                                                               | g./l. |
|---------------------------------------------------------------|-------|
| Nickel sulfate ( $\text{NiSO}_4 \cdot 6\text{H}_2\text{O}$ )  | 300.0 |
| Nickel chloride ( $\text{NiCl}_2 \cdot 6\text{H}_2\text{O}$ ) | 37.5  |
| Boric acid ( $\text{H}_3\text{BO}_3$ )                        | 37.5  |
| pH of bath 3.49 at 27.5° C.                                   |       |

A solution in the amount of 10 grams of sodium carboxymethylcellulose (medium viscosity grade) and 1 liter of distilled water was then made up by mixing in a Waring Blender. This latter solution was then added to the first prepared electroplating solution, in varying proportions. Specimen brass test plates 1 and  $\frac{1}{2}$  inches wide by 3 inches long, and 0.025 inch thickness, were then immersed in the so-prepared solution and electroplated for 11½ minutes at a current density of 50 amperes per square foot. The approximate depth of the nickel plate deposited upon the brass specimens was 0.0005 inch. The electroplating solutions were maintained at a temperature of  $135^\circ \pm 2^\circ \text{ F}$ . Two series of electroplating runs were made: one series in a still bath where there was no agitation or stirring, and the other series where the specimen being plated was moved backwards and forwards in a line parallel to the surface of the electrodes at a linear speed of 15 feet per minute. After removal from the plating solution, the plates were then dried and their brightness measured by a reflectometer. The results obtained are tabulated as follows:

2  
Table I  
NICKEL PLATING BATH

| 5  | Amount (in cc.) of carboxymethylcellulose solution per liter plating solution | Percent by weight of sodium carboxymethylcellulose present | Reflectance |          | Percent Increase in Reflectance |          |
|----|-------------------------------------------------------------------------------|------------------------------------------------------------|-------------|----------|---------------------------------|----------|
|    |                                                                               |                                                            | Still       | Agitated | Still                           | Agitated |
| 10 | 0                                                                             | 0.0                                                        | 27          | 31       |                                 |          |
|    | 1                                                                             | 0.001                                                      | 29          | 30       | 7                               | -3       |
|    | 2                                                                             | 0.002                                                      | 29          | 35       | 7                               | 13       |
|    | 5                                                                             | 0.005                                                      | 36          | 40       | 33                              | 29       |
| 10 | 10                                                                            | 0.01                                                       | 36          | 62       | 33                              | 100      |
| 20 | 20                                                                            | 0.02                                                       | 55          | 73       | 104                             | 132      |
| 50 | 50                                                                            | 0.05                                                       | 71          | 71       | 163                             | 129      |
| 15 | 100                                                                           | 0.10                                                       | 71          | 68       | 163                             | 120      |

From the foregoing results it will be seen that the sodium carboxymethylcellulose addition imparts a marked increase in brightness, on the order of one-third improvement, in both the still and agitated baths, beginning at 0.005% addition to the nickel electroplating solution. At 0.05% addition the increase in brightness reaches a maximum and levels off.

## EXAMPLE 2

A cadmium plating bath solution was made up as follows:

|                                  | G./l. |
|----------------------------------|-------|
| Sodium cyanide ( $\text{NaCN}$ ) | 525   |
| Cadmium oxide ( $\text{CdO}$ )   | 135   |

The same grade of sodium carboxymethylcellulose as used in Example 1, was added in varying proportions to the so-prepared cadmium plating bath. Similar brass specimens were then subjected to an electroplating procedure for a period of 9.73 minutes at a current density of 30 amperes per square foot, producing an electroplate thickness of approximately 0.0005 in. The temperature of the bath was maintained at  $80^\circ \pm 2^\circ \text{ F}$ . The brightness of the several cadmium plate specimens, plated in a still bath, was then ascertained as set forth in the following table:

45  
Table II  
CADMIUM PLATING BATH

|    | Percent by weight of sodium carboxymethylcellulose present | Reflectance (Still Bath) | Percent Increase in Reflectance |
|----|------------------------------------------------------------|--------------------------|---------------------------------|
| 50 | 0.0                                                        |                          |                                 |
|    | 0.1                                                        | 8                        |                                 |
|    | 0.2                                                        | 14                       | 75                              |
|    | 0.5                                                        | 36                       | 350                             |
|    |                                                            | 21                       | 163                             |

From the above results it will be seen that a relatively larger addition of sodium carboxymethylcellulose is required to obtain the brightening effect in the cadmium plating bath as compared to the nickel plating bath. In other words the increase in brightness is first manifest at 0.1% addition of sodium carboxymethylcellulose, reaching a maximum at 0.2% and leveling off or slightly decreasing from such maximum thereafter. The sodium carboxymethylcellulose addition may be increased up to 2.5% in the cadmium plating bath while still retaining a brightness increase, as compared to the bath with no such addition.

Other modes of applying the principle of my invention may be employed, changes being made as regards to the details described, provided the features stated in any of the following claims or the equivalent of such be employed.

I, therefore, particularly point out and distinctly claim as my invention:

1. An electroplating bath comprising an aqueous solution of sodium cyanide, cadmium oxide, and containing an addition of 0.1-2.5% of sodium carboxymethylcellulose, on the solution weight basis.
2. An electroplating bath comprising an aqueous solution of nickel sulfate, nickel chloride, boric acid, and containing an addition of 0.05-0.10% of sodium carboxymethylcellulose, on the solution weight basis.
3. An electroplating bath comprising an aqueous solution of sodium cyanide, cadmium oxide, and containing an addition of 0.1-0.5% of sodium carboxymethylcellulose, on the solution weight basis.

4. An electroplating bath comprising an aqueous solution of inorganic metallic compounds selected from the group consisting of an acid solution of a mixture of nickel chloride and nickel sulfate salts, and an alkaline cyanide solution of cadmium oxide; and containing an addition of sodium carboxymethylcellulose ranging, on the solution weight basis, from 0.05-0.10% when the nickel bath is employed and from 0.1-2.5% when the cadmium bath is used.

5. The process of brightening deposits of nickel and cadmium in electroplating baths selected from the group consisting of an acid solution of a mixture of nickel chloride and nickel sulfate salts and an alkaline cyanide solution of cadmium oxide, which comprises adding 0.05-2.50% by weight of sodium carboxymethylcellulose to the bath.

ANDREW W. LIGER.

#### REFERENCES CITED

The following references are of record in the file of this patent:

#### UNITED STATES PATENTS

| Number    | Name   | Date          |
|-----------|--------|---------------|
| 1,564,414 | Hoff   | Dec. 8, 1925  |
| 2,061,592 | Rapids | Nov. 24, 1936 |

#### OTHER REFERENCES

Chemical Trade Journal and Chemical Engineering, January 4, 1946, pages 7-8.  
Metal Finishing, June 1940, pages 315-17.